# EUROPEAN PATENT SPECIFICATION

(11) **EP 2 886 675 B1**
(45) Date of publication and mention of the grant of the patent: **22.05.2019**
(21) Application number: 14199446.7
(22) Date of filing: 19.12.2014
(51) Int. Cl.: C22C 38/58, C22C 38/42, C22C 38/34, C22C 38/46, C22C 38/44, C22C 38/48, C22C 38/00, C22C 38/02, C21D 6/00, C21D 8/02, C21D 1/18, C22C 38/06, C22C 38/50, C22C 38/52

(54) **High strength steel alloy and strip and sheet product made therefrom**
Hochfeste Stahllegierung und daraus hergestelltes Band- und Blechprodukt
Alliage d'acier à haute résistance et feuille de bande et produit fabriqué à partir de celui-ci

(30) Priority: 20.12.2013 US 201361919081 P
(43) Date of publication of application: 24.06.2015
(73) Proprietor: CRS Holdings, Inc., Wilmington DE 19801 (US)
(72) Inventor: Novotny, Paul M., Mohnton, Pennsylvania 19540 (US)
(74) Representative: Mewburn Ellis LLP

(56) References cited:
- EP-A1- 1 975 266
- EP-A1- 2 397 571
- EP-A1- 2 543 747
- WO-A1-2012/153831
- JP-A- H11 229 075
- JP-A- H11 269 541
- JP-A- 2010 116 593
- JP-A- 2012 001 802
- US-B1- 7 067 019

## Description

### BACKGROUND OF THE INVENTION

### FIELD OF THE INVENTION

This invention relates to a steel alloy having a unique combination of high strength, high toughness, and high ductility. The invention also relates to the use of the steel alloy to make thin gauge product forms such as strip and sheet that can be readily formed into parts for automotive use.

### DESCRIPTION OF THE RELATED ART

The US Environmental Protection Agency requires that new cars must meet a 23.2 km/l (54.5 miles/gallon) corporate average fuel economy standard by the year 2025. This requirement will likely cause automobile manufacturers to reduce the weights of their vehicles. Light-weight materials such as aluminum and composite materials that provide high strength and significant reduction in weight compared to the known steel alloys can be used for making thin-gauge auto body and frame parts. However, the use of such materials will present challenges to auto manufacturers because their production line-ups are designed for using steel alloys and a change to non-steel materials such as aluminum and composites would require substantial capital investments as well as a substantial increase in the cost of materials.

Steel sheet and strip that provide higher strength than conventional steels used for auto body and frame applications can be used to reduce the weight of stamped body and frame parts in this "Light Weighting" effort as long as they are sufficiently tough and formable. A measure of the strength and formability of a steel is a Strip Index Number (SIN) which is the product of the ultimate tensile strength (UTS) in MPa and the Elongation in %. For many automotive applications steel sheet and strip having an SIN of at least about 20,000 provide sufficient weight reduction while providing adequate strength and formability. However, for structural parts that require higher strength, an SIN of at least about 30,000 is preferred. Many of the steels known as advanced high strength steels (AHSS) leave something to be desired with respect to ductility because strength and ductility are inversely related properties. Good ductility is needed for strip and sheet forms of high strength steel material to provide good formability. Accordingly, it would be desirable to have a steel alloy that provides a combination of high strength and ductility that not only results in significant weight reduction in automotive body and frame parts, but also can be readily formed into such products.

US 7,067,019 describes a relatively high strength high toughness medium Carbon Copper-Nickel-Chromium alloy steel and method of making the steel.

EP 2 543 747 A1 discloses a seamless steel pipe for a high-strength hollow spring.

JP H11-269541 discloses a high strength steel having improved resistance to crack propagation and a method of making the steel.

### SUMMARY OF THE INVENTION

The foregoing need is resolved to a large degree by a steel alloy in accordance with the present invention. The alloy according to this invention provides a unique combination of very high strength, toughness, and ductility. The alloy of this invention can be characterized by the broad, intermediate and preferred weight percent compositions set forth below.

| **Element** | **Broad** | **Intermediate** | **Preferred A** | **Preferred B** |
|---|---|---|---|---|
| **C** | 0.3-0.45 | 0.30-0.45 | 0.30-0.40 | 0.30-0.36 |
| **Mn** | 3.5-4.5 | 3.5-4.5 | 3.5-4.5 | 3.5-4.5 |
| **Si** | 1.0-2.0 | 1.3-1.8 | 1.3-1.7 | 1.3-1.7 |
| **Cr** | 0.6-2.5 | 0.75-2.35 | 1.6-2.35 | 0.75-1.5 |
| **Ni** | 0.6-5.0 | 0.7-4.5 | 3.7-4.3 | 0.7-2.5 |
| **Mo+½W** | Up to 0.5 | Up to 0.3 | 0.1 max. | 0.15-0.25 |
| **Cu** | 0.3-1.0 | 0.4-0.7 | 0.4-0.6 | 0.4-0.6 |
| **Co** | 0.01 max. | 0.01 max. | 0.01 max. | 0.01 max. |
| **V+5/9Nb** | 0.1-0.5 | 0.2-0.4 | 0.30-0.40 | 0.20-0.30 |
| **Ti** | 0.025 max. | 0.020 max. | 0.020 max. | 0.020 max. |
| **Al** | 0.025 max. | 0.020 max. | 0.020 max. | 0.020 max. |
| **Ca** | 0.005 max. | 0.002 max. | 0.001 max. | 0.001 max. |
| **N** | 0.020 max. | 0.020 max. | 0.020 max. | 0.020 max. |

The alloy may optionally include one or both of 0.001-0.025% Y and 0.001-0.01% Mg. The balance of the alloy is iron and the usual impurities found in commercial grades of steel alloys produced for similar use and properties. Among said impurities phosphorus is preferably restricted to not more than about 0.03% max. and sulfur is preferably restricted to not more than about 0.003% max. Within the foregoing ranges, the elements Si, Cu, V, and when present, Nb are balanced such that 4.5 ≤ (%Si + %Cu)/(%V + (5/9) × %Nb) ≤ 10.

The foregoing tabulation is provided as a convenient summary and is not intended to restrict the lower and upper values of the ranges of the individual elements for use in combination with each other, or to restrict the ranges of the elements for use solely in combination with each other. Thus, one or more of the ranges can be used with one or more of the other ranges for the remaining elements. In addition, a minimum or maximum for an element of a broad or preferred composition can be used with the minimum or maximum for the same element in another preferred or intermediate composition. Moreover, the alloy according to the present invention may comprise, consist essentially of, or consist of the constituent elements described above and throughout this application. Here and throughout this specification the term "percent" or the symbol "%" means percent by weight or mass percent, unless otherwise specified. Furthermore, the term "about" used in connection with a weight percent value or range means the usual analytical tolerance or experimental error expected by a person skilled in the art based on known, standardized measuring techniques.

In accordance with another aspect of this invention, there is provided a thin gauge steel product such as sheet or strip product that is made from one of the steel alloys described in the table. The thin gauge products can be readily formed into automotive parts because of their good ductility. A thin gauge steel product in accordance with this aspect of the invention has an SIN of at least about 20,000 and better yet, and SIN of at least 25,000. A preferred embodiment of the steel product has an SIN of at least about 30,000.

### DETAILED DESCRIPTION

The invention is defined in the claims.

The weight percent ranges described above can be further defined by the roles the elements play in the alloy of this invention. The combination of the elements silicon, copper, and vanadium, and niobium when present, function as diffusion modifiers for the purposes of this invention because they have been shown to reduce the diffusion of carbon as well as deleterious tramp elements such as P and S to the grain boundaries of the alloy. Molybdenum is optionally present in the alloy according to this invention and tungsten may be substituted for some or all of the molybdenum in this alloy. When present, tungsten is substituted for molybdenum on a 2:1 basis such that Mo+ ½W is about 0.20-0.5% and preferably about 0.15-0.3%. Yttrium and magnesium may also be present in this alloy either separately or in combination. In this regard the alloy may contain about 0.001-0.025% yttrium and preferably may contain about 0.002-0.020% yttrium. The alloy may also contain about 0.001-0.01% magnesium and preferably may contain about 0.001-0.006% magnesium. The magnesium and/or yttrium is added during primary melting to deoxidize the steel alloy. Magnesium and yttrium also benefit the strength and toughness of this steel by aiding in grain refinement of the alloy during processing.

The elements molybdenum, tungsten, and chromium combine with carbon to form M₂C carbides (where M is Cr, Mo, and/or W) during tempering. The elements Mo, W, and Cr can be referred to as tempered carbide formers for the purposes of the alloy according to this invention. Thus, chromium and molybdenum and tungsten when present, promote the formation of M₂C carbides and can be substituted for each other in this alloy. For thin gauge product forms such as strip and sheet where an SIN of at least 30,000 is desired, a positive addition of molybdenum and or tungsten is included as described above. Further, within the foregoing weight percent ranges, molybdenum, chromium, and carbon are preferably balanced such that 3.5 ≤ (%Mo +% Cr)/(%C) ≤ 7.5.

The elements manganese and nickel are austenite stabilizers and contribute to the good hardenability of this alloy. Manganese and nickel can be substituted for each other to a limited extent to stabilize austenite. For the thin gauge product applications where an SIN of at least about 30,000 is desired, within the foregoing weight percent ranges, manganese and nickel are broadly balanced such that 3.5 ≤ (%Mn + %Ni) ≤ 8.0.

This alloy and products made therefrom are preferably prepared by vacuum melting techniques. In this regard, primary melting of the alloy is preferably accomplished with vacuum induction melting (VIM). When desired, as for more critical applications, the alloy can be refined using vacuum arc remelting (VAR). Primary melting may also be performed by arc melting in air (ARC) if desired. After ARC melting, the alloy may be refined by electroslag remelting (ESR) or VAR.

The alloy of this invention is preferably processed to thin gauge forms such as strip or sheet. In strip or sheet form, parts made from the alloy can be austenitized for short times at a temperature of about 760 to 1038°C (1400 to 1900°F) and then air cooled. The parts can then be used in service. Alternatively, annealed strip or sheet can be formed into a shaped part and then regions of the part can be selectively heat treated by induction heating to the austenitizing temperature of 760 to 1038°C (1400 to 1900°F) followed by cooling in air. Another option is to heat the strip or sheet material to the austenitizing temperature of 760 to 1038°C (1400 to 1900°F) then stamp the part to form it and allow the hot stamped part to air cool. The parts can be used in the air-cooled condition or after short time tempers at 204.4-371°C (400 to 700°F). The alloy has relatively high ultimate tensile strength (UTS) in the annealed condition, i.e., at least about 1025 MPa (150 ksi) on average, combined with very high ductility (i.e., 10-25% Elongation). Therefore, parts made from annealed alloy strip or sheet may be used in some applications without any further heat treatment.

The alloy may also be hot worked from a temperature of up to about 1149°C (2100°F), preferably at about 982°C (1800°F), to form various intermediate product forms such as billets and bars. The alloy is preferably heat treated by austenitizing at about 863°C (1585°F) to about 1002°C (1835°F) for about 1-2 hours. The alloy is then air cooled or oil quenched from the austenitizing temperature. When desired, the alloy can be vacuum heat treated and gas quenched. Parts made from the alloy in bar form are preferably deep chilled at either -73.3°C (-100°F) or -196°C (-320°F) for about 1-8 hours and then warmed in air. If lower strength is acceptable the refrigeration step may be eliminated for parts made from bar products. The alloy is preferably tempered at about 204.4 to 316°C (400°F to 600°F) for about 2-3 hours and then air cooled. The alloy may be tempered at up to 371°C (700°F) when an optimum combination of strength and toughness is not required.

In accordance with a further aspect of the present invention there is provided a shaped part made from a thin gauge product form of the alloy as described above. The shaped part is preferably embodied as a stamped body or frame part for an automobile. A thin gauge product in accordance with the present invention is a part or component made from sheet or strip having a thickness of at least about 0.0229 mm (0.0009 in.) and less than 6.35 mm (0.25 in.).

### WORKING EXAMPLES

### Example I

To demonstrate the unique combination of properties provided by the alloy according to the present invention, representative examples of the alloy and examples of comparative alloys were melted, processed, and tested. The weight percent compositions of the tested alloys are set forth in Table 1 below. Example 1 represents the alloy according to the present invention. Alloys A, B, and C are comparative alloys.

**TABLE 1**

| **Element** | | **Example 1** | **Alloy A** | **Alloy B** | **Alloy C** |
|---|---|---|---|---|---|
| **C** | | 0.36 | 0.48 | 0.38 | 0.51 |
| **Mn** | | 4.02 | 6.88 | 4.71 | 0.68 |
| **Si** | | 1.44 | 1.43 | 1.70 | 1.45 |
| **Cr** | | 1.98 | 1.99 | 1.60 | 1.98 |
| **Ni** | | 3.96 | 0.70 | 3.88 | 6.85 |
| **Mo** | | --- | --- | 0.12 | --- |
| **Cu** | | 0.52 | 0.64 | 0.66 | 0.64 |
| **V** | | 0.36 | 0.21 | 0.30 | 0.22 |

The balance of each composition in Table 1 is iron and impurities.

The examples and comparative alloys were vacuum induction melted and cast as 15.9 kg (35 lb.) heats. The heats were hot worked and rough machined into sets of duplicate standard tensile specimens. The pairs of specimens from each set were austenitized at different temperatures for 1.5 hours and then oil quenched. The specimen pairs were then tempered for 2 hours and air cooled. The combinations of austenitizing temperature and tempering temperature used for the specimen pairs of each alloy are set forth in Table 2 below.

**TABLE 2**

| **Heat Treatment ID** | **Austenitizing Temperature** | **Tempering Temperature** |
|---|---|---|
| **A** | 890.6°C (1635°F) | 204°C (400°F) |
| **B** | 890.6°C (1635°F) | 316°C (600°F) |
| **C** | 918.3°C (1685°F) | 204°C (400°F) |
| **D** | 918.3°C (1685°F) | 260°C (500°F) |
| **E** | 946.1°C (1735°F) | 204°C (400°F) |

After heat treatment, the test specimens were finish machined to final dimension and tested. The results of room temperature tensile tests for each example are presented in Tables 3A to 3D below including the 0.2% offset yield strength (Y.S.), the ultimate tensile strength (U.T.S.), the percent elongation (% El.), and the percent reduction in area (%R.A.). Also included in the tables are calculations of the SIN for each specimen (SIN = UTS in MPa x % El.). Average values for each pair of the tested specimens are also presented in the tables.

**TABLE 3A**

| | | | | **Y.S.** | **U.T.S.** | | **%EL.** | **%R.A.** | **SIN** |
|---|---|---|---|---|---|---|---|---|---|
| **Heat ID** | **Heat Treatment** | **Sample** | **ksi** | MPa | **(ksi)** | (MPa) | | | |
| **Example 1** | **A** | A1 | 121.3 | 836.4 | 284.4 | 1960.9 | 15.8 | 19.0 | **30,903** |
| | | A2 | 125.3 | 863.6 | 285.0 | 1965.2 | 17.1 | 28.9 | **33,546** |
| | | **Avg.** | **123.3** | **850.0** | **284.7** | **1963.1** | **16.4** | **24.0** | **32,225** |
| | | | | | | | | | |
| | **B** | B1 | 139.6 | 962.5 | 240.8 | 1660.3 | 19.4 | 21.8 | **32,211** |
| | | B2 | 143.6 | 990.4 | 239.1 | 1648.8 | 21.4 | 18.3 | **35,285** |
| | | **Avg.** | **141.6** | **976.4** | **240.0** | **1654.6** | **20.4** | **20.0** | **33,748** |
| | | | | | | | | | |
| | **C** | C1 | 121.7 | 839.2 | 285.3 | 1966.7 | 15.7 | 23.9 | **30,878** |
| | | C2¹ | | | | | | | |
| | | **Avg.** | **121.7** | **839.2** | **285.3** | **1966.7** | **15.7** | **23.9** | **30,878** |
| | | | | | | | | | |
| | **D** | D1 | 124.6 | 859.4 | 264.6 | 1824.1 | 17.3 | 25.4 | **31,557** |
| | | D2 | 128.9 | 888.5 | 263.1 | 1814.2 | 21.4 | 28.1 | **38,824** |
| | | **Avg.** | **126.8** | **874.0** | **263.8** | **1819.2** | **19.4** | **26.7** | **35,191** |
| | | | | | | | | | |
| | **E** | E1 | 111.8 | 770.9 | 289.5 | 1996.2 | 13.7 | 13.2 | **27,348** |
| | | E2 | 115.2 | 794.0 | 289.3 | 1994.9 | 14.8 | 17.6 | **29,525** |
| | | **Avg.** | **113.5** | **782.5** | **289.4** | **1995.6** | **14.3** | **15.4** | **28,436** |

| | | | | | | | | | |
|---|---|---|---|---|---|---|---|---|---|
| ¹ Sample not tested because of forging defect. | | | | | | | | | |

**TABLE 3B**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Alloy A** | **A** | A1 | 61.9 | 426.7 | 100.6 | 693.7 | 8.8 | 8.6 | **6,104** |
| | | A2 | 60.8 | 418.9 | 115.7 | 797.5 | 9.5 | 8.5 | **7,568** |
| | | **Avg.** | **61.3** | **422.8** | **108.1** | **745.6** | **9.1** | **8.5** | **6,836** |
| | | | | | | | | | |
| | **B** | B1 | 67.0 | 461.8 | 132.2 | 911.6 | 9.7 | 8.0 | **8,843** |
| | | B2 | 65.2 | 449.4 | 154.9 | 1067.7 | 11.8 | 9.4 | **12,598** |
| | | **Avg.** | **66.1** | **455.6** | **143.5** | **989.6** | **10.8** | **8.7** | **10,721** |
| | | | | | | | | | |
| | **C** | C1 | 62.8 | 433.1 | 146.3 | 1008.5 | 11.6 | 11.5 | **11,699** |
| | | C2 | 63.0 | 434.1 | 132.3 | 912.4 | 12.1 | 11.5 | **11,040** |
| | | **Avg.** | **62.9** | **433.6** | **139.3** | **960.4** | **11.9** | **11.5** | **11,369** |
| | | | | | | | | | |
| | **D** | D1 | 65.0 | 448.4 | 140.0 | 965.5 | 12.5 | 10.7 | **12,068** |
| | | D2 | 62.9 | 433.5 | 127.6 | 879.7 | 10.1 | 10.8 | **8,885** |
| | | **Avg.** | **64.0** | **441.0** | **133.8** | **922.6** | **11.3** | **10.7** | **10,477** |
| | | | | | | | | | |
| | **E** | E1 | 59.6 | 411.1 | 132.8 | 915.5 | 12.0 | 12.4 | **10,986** |
| | | E2 | 57.3 | 395.1 | 117.4 | 809.7 | 10.7 | 11.5 | **8,663** |
| | | **Avg.** | **58.5** | **403.1** | **125.1** | **862.6** | **11.4** | **12.0** | **9,825** |

**TABLE 3C**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Alloy B** | **A** | A1 | 55.9 | 385.1 | 221.2 | 1525.2 | 6.7 | 6.5 | **10,265** |
| | | A2 | 64.5 | 444.6 | 212.4 | 1464.1 | 6.7 | 5.9 | **9,853** |
| | | **Avg.** | **60.2** | **414.8** | **216.8** | **1494.7** | **6.7** | **6.2** | **10,059** |
| | | | | | | | | | |
| | **B** | B1 | 91.7 | 632.2 | 220.5 | 1520.0 | 5.5 | 9.3 | **8,360** |
| | | B2 | 79.5 | 547.9 | 208.6 | 1438.4 | 5.8 | 13.2 | **8,343** |
| | | **Avg.** | **85.6** | **590.1** | **214.5** | **1479.2** | **5.7** | **11.2** | **8,351** |
| | | | | | | | | | |
| | **C** | C1 | 70.4 | 485.4 | 188.6 | 1300.4 | 4.9 | 4.1 | **6,372** |
| | | C2 | 68.5 | 472.5 | 210.0 | 1447.8 | 5.5 | 4.0 | **7,963** |
| | | **Avg.** | **69.5** | **478.9** | **199.3** | **1374.1** | **5.2** | **4.1** | **7,168** |
| | | | | | | | | | |
| | **D** | D1 | 68.3 | 471.1 | 195.6 | 1348.3 | 5.5 | 4.9 | **7,416** |
| | | D2 | 66.9 | 461.5 | 219.3 | 1512.0 | 6.7 | 8.4 | **10,130** |
| | | **Avg.** | **67.6** | **466.3** | **207.4** | **1430.2** | **6.1** | **6.7** | **8,773** |
| | **E** | E1 | 53.2 | 366.9 | 162.1 | 1117.6 | 3.7 | 3.3 | **4,135** |
| | | E2 | 49.8 | 343.4 | 139.4 | 961.1 | 3.8 | 3.3 | **3,652** |
| | | **Avg.** | **51.5** | **355.2** | **150.7** | **1039.4** | **3.8** | **3.3** | **3,894** |

**TABLE 3D**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Alloy** C | A | A1 | 186.7 | 1287.5 | 300.7 | 2072.9 | 17.7 | 32.7 | **36,691** |
| | | A2 | 184.8 | 1274.2 | 301.6 | 2079.3 | 14.4 | 23.2 | **29,942** |
| | | **Avg.** | **185.8** | **1280.8** | **301.1** | **2076.1** | **16.1** | **27.9** | **33,317** |
| | | | | | | | | | |
| | **B** | B1 | 192.0 | 1323.7 | 255.7 | 1762.7 | 15.3 | 31.4 | **26,969** |
| | | B2 | 196.0 | 1351.5 | 256.7 | 1770.1 | 18.5 | 39.6 | **32,747** |
| | | **Avg.** | **194.0** | **1337.6** | **256.2** | **1766.4** | **16.9** | **35.5** | **29,858** |
| | | | | | | | | | |
| | **C** | C1 | 164.4 | 1133.4 | 304.5 | 2099.5 | 14.4 | 18.2 | **30,233** |
| | | C2 | 165.0 | 1137.4 | 304.0 | 2096.0 | 15.4 | 18.3 | **32,278** |
| | | **Avg.** | **164.7** | **1135.4** | **304.3** | **2097.7** | **14.9** | **18.3** | **31,255** |
| | | | | | | | | | |
| | **D** | D1 | 173.3 | 1194.8 | 274.1 | 1890.1 | 16.1 | 21.8 | **30,431** |
| | | D2 | 177.0 | 1220.3 | 274.5 | 1892.4 | 19.3 | 39.6 | **36,524** |
| | | **Avg.** | **175.1** | **1207.6** | **274.3** | **1891.3** | **17.7** | **30.7** | **33,477** |
| | | | | | | | | | |
| | **E** | E1 | 151.5 | 1044.4 | 304.0 | 2095.7 | 15.4 | 21.1 | **32,273** |
| | | E2 | 162.3 | 1119.2 | 304.3 | 2097.7 | 18.0 | 35.8 | **37,759** |
| | | **Avg.** | **156.9** | **1081.8** | **304.1** | **2096.7** | **16.7** | **28.5** | **35,016** |

### Example II

In order to demonstrate that the alloy of the present invention is capable of providing the desired combination of properties when scaled up to commercial production-size heats, two additional heats were melted, processed, and tested. The weight percent compositions of the tested alloys are set forth in Table 4 below. Example 2 represents the alloy according to the Preferred A composition of the alloy according to the present invention and Example 3 represents the alloy according to the Preferred B composition of the alloy according to the present invention.

**TABLE 4**

| **Element** | **Example 2** | **Example 3** |
|---|---|---|
| **C** | 0.357 | 0.311 |
| **Mn** | 4.01 | 4.04 |
| **Si** | 1.54 | 1.57 |
| **P** | 0.018 | 0.015 |
| **S** | <0.0005 | <0.0005 |
| **Cr** | 2.05 | 1.11 |
| **Ni** | 4.02 | 0.96 |
| **Mo** | 0.03 | 0.20 |
| **Cu** | 0.51 | 0.51 |
| **V** | 0.36 | 0.24 |
| **Ti** | 0.0050 | 0.0040 |
| **Al** | 0.0020 | 0.0060 |
| **N** | 0.0044 | 0.0041 |
| **Ca** | 0.0015 | 0.0016 |

The balance of each composition in Table 4 is iron and impurities.

Examples 2 and 3 were melted and refined by ARC and AOD as 36.29-Mg (40-ton) heats and then cast as billet on a continuous caster. The continuously cast billets were hot worked and rough machined into sets of duplicate standard tensile specimens. Duplicate tensile test specimens for Example 2 were prepared from 3.81 mm (0.150 inch) thick hot rolled band. Duplicate tensile test specimens for Example 3 were prepared from 3.81 mm (0.150 inch) thick hot rolled band as follows. A first set of specimens were prepared from the 3.81 mm (0.150 in.) band after grinding the band material to a final thickness of 2.8 mm (0.110 in.). A second set of specimens were prepared by cold rolling the 3.81 mm (0.150 in.) band material to form strip having a thickness of 3.3 mm (0.130 in.). The strip material was ground to a final thickness of 2.2 mm (0.087 in.). A third set of specimens were prepared by cold rolling the band material to form strip having a thickness of 2.8 mm (0.110 in.) and then grinding the strip material to a final thickness of 1.9 mm (0.074 in.).

The pairs of the tensile specimens of Example 2 were heat treated by placing the specimens into stainless steel bags which were then backfilled with argon gas and divided into subsets. Each subset was heat treated in accordance with one of the heat treatments A-H set forth in Table 2 above. Austenitizing was performed by holding the specimen subset at temperature for 1.5 hours and then oil quenching to room temperature. Tempering was performed by holding the specimen subset at the respective tempering temperature for 2 hours followed by air cooling to room temperature.

The pairs of tensile specimens of Example 3 were heat treated in three groups. One group was heat treated with Heat Treatment A in Table 2 above. A second group was heat treated with Heat Treatment C of Table 2 and the third group was heat treated with Heat Treatment E of Table 2. Austenitizing was performed by holding the specimens at the respective temperature for 1.5 hours and then air cooling to room temperature. Tempering was performed by holding the specimens at the respective tempering temperature for 2 hours followed by air cooling to room temperature.

The results of room temperature tensile tests for Example 2 are presented in Table 5 below including the 0.2% offset yield strength (Y.S.), the ultimate tensile strength (U.T.S.), the percent elongation (% El.), and the percent reduction in area (%R.A.). Also included in the tables are calculations of the SIN for each specimen (SIN = UTS in MPa x % El.). Average values for each pair of the tested specimens are also presented in the tables.

**TABLE 5**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Example 2** | **A** | A1 | 150.2 | 1035.5 | 267.9 | 1846.8 | 17.0 | 38.8 | **31,395** |
| | | A2 | 141.9 | 978.3 | 271.6 | 1872.6 | 18.0 | 21.3 | **33,707** |
| | | **Avg.** | **146.0** | **1006.9** | **269.7** | **1859.7** | **17.5** | **30.0** | **32,551** |
| | | | | | | | | | |
| | **B** | B1 | 161.2 | 111.2 | 230.7 | 1590.5 | 21.3 | 42.7 | **33,877** |
| | | B2 | 159.9 | 1102.5 | 228.9 | 1578.2 | 20.2 | 31.3 | **31,879** |
| | | **Avg.** | **160.5** | **1106.9** | **229.8** | **1584.6** | **20.8** | **37.0** | **32,878** |
| | | | | | | | | | |
| | **C** | C1 | 143.3 | 987.7 | 269.2 | 1856.4 | 17.9 | 31.3 | **33,229** |
| | | C2 | 139.7 | 963.0 | 267.7 | 1845.8 | 20.1 | 39.2 | **37,101** |
| | | **Avg.** | **141.5** | **975.4** | **268.5** | **1851.1** | **19.0** | **35.2** | **35,165** |
| | | | | | | | | | |
| | **D** | D1 | 146.6 | 1010.8 | 250.1 | 1724.4 | 20.6 | 36.6 | **35,522** |
| | | D2 | 156.5 | 1079.0 | 245.4 | 1691.8 | 20.0 | 39.1 | **33,837** |
| | | **Avg.** | **151.6** | **1044.9** | **247.7** | **1708.1** | **20.3** | **37.8** | **34,680** |
| | | | | | | | | | |
| | **E** | E1 | 141.9 | 978.6 | 265.6 | 1831.1 | 17.6 | 35.7 | **32,264** |
| | | E2 | 137.5 | 948.0 | 275.1 | 1896.8 | * | 36.7 | ** |
| | | **Avg.** | **139.7** | **963.3** | **270.3** | **1864.0** | **17.6** | **36.2** | **32,264** |
| | | | | | | | | | |
| | **F** | **F1** | 146.0 | 1006.5 | 243.0 | 1675.4 | 22.4 | 43.9 | 37,528 |
| | | **F2** | 147.2 | 1014.8 | 245.0 | 1689.2 | * | 40.4 | ** |
| | | **Avg.** | **146.6** | **1010.6** | **244.0** | **1682.3** | **22.4** | **42.2** | **37,528** |
| | | | | | | | | | |
| | **G** | **G1** | 130.0 | 896.1 | 266.9 | 1840.5 | 17.9 | 29.1 | 32,945 |
| | | **G2** | 131.1 | 904.0 | 268.5 | 1851.4 | 17.8 | 24.4 | 32,584 |
| | | **Avg.** | **130.5** | **900.0** | **267.7** | **1845.9** | **17.8** | **26.8** | **32,765** |
| | | | | | | | | | |
| | **H** | **H1** | 137.3 | 946.7 | 262.4 | **1808.9** | 20.6 | 39.7 | 37,264 |
| | | **H2** | 136.8 | 942.9 | 267.8 | 1846.4 | * | 32.9 | ** |
| | | **Avg.** | **137.0** | **944.8** | **265.1** | **1827.7** | **20.6** | **36.3** | **37,264** |

| | | | | | | | | | |
|---|---|---|---|---|---|---|---|---|---|
| * = Invalid measurement - Specimen broke outside gage section ** = No value could be calculated. | | | | | | | | | |

The results of room temperature tensile tests for Example 3 are presented in Tables 6A, 6B, and 6C below.

**TABLE 6A**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Example 3 Group 1** | **A** | A1 | 174.0 | 1199.4 | 266.6 | 1837.9 | * | * | ** |
| | | A2 | 173.9 | 1199.1 | 257.1 | 1772.3 | 13.9 | 41.3 | **24,635** |
| | | **Avg.** | **173.9** | **1199.2** | **261.8** | **1805.1** | **13.9** | **41.3** | **24,635** |
| | | | | | | | | | |
| | **C** | C1 | 164.8 | 1136.3 | 253.4 | 1746.9 | 14.0 | 32.7 | **24,457** |
| | | C2 | 169.0 | 1165.4 | 257.7 | 1776.9 | 14.6 | 23.2 | **25,924** |
| | | **Avg.** | **166.9** | **1150.8** | **255.5** | **1761.9** | **14.3** | **27.9** | **25,191** |
| | | | | | | | | | |
| | **E** | E1 | 164.4 | 1133.4 | 257.3 | 1774.0 | 13.1 | 39.5 | **23,240** |
| | | E2 | 172.5 | 1189.3 | 262.9 | 1812.6 | 13.0 | 35.5 | **23,492** |
| | | **Avg.** | **168.4** | **1161.4** | **260.1** | **1793.3** | **13.0** | **37.5** | **23,366** |

| | | | | | | | | | |
|---|---|---|---|---|---|---|---|---|---|
| * = Invalid measurement - Specimen broke outside gage section ** = No value could be calculated. | | | | | | | | | |

**TABLE 6B**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Example 3** | **A** | A1 | 179.4 | 1237.2 | 262.3 | 1808.4 | * | 33.2 | *** |
| **Group 2** | | A2 | 177.3 | 1222.4 | 253.3 | 1746.2 | * | 41.9 | *** |
| | | **Avg.** | **178.4** | **1229.3** | **257.8** | **1777.3** | | **37.5** | |
| | | | | | | | | | |
| | **C** | C1** | | | | | | | |
| | | C2 | 175.1 | 1207.4 | 263.2 | 1814.6 | * | 43.2 | *** |
| | | **Avg.** | **175.1** | **1207.4** | **263.2** | **1814.6** | | **43.2** | |
| | | | | | | | | | |
| | **E** | E1 | 171.0 | 1178.7 | 266.3 | 1836.2 | * | 36.9 | *** |
| | | E2 | 176.4 | 1215.9 | 265.2 | 1828.4 | 13.1 | 36.8 | **23,934** |
| | | **Avg.** | **173.7** | **1197.3** | **265.8** | **1832.3** | **13.1** | **36.8** | **23,934** |

| | | | | | | | | | |
|---|---|---|---|---|---|---|---|---|---|
| * = Invalid measurement - Specimen broke outside gage section. ** = No test because sample was damaged during processing. *** = No value could be calculated. | | | | | | | | | |

**TABLE 6C**

| | | | **Y.S.** | | **U.T.S.** | | **%EI.** | **%R.A.** | **SIN** |
|---|---|---|---|---|---|---|---|---|---|
| **Heat ID** | **Heat Treatment** | **Sample** | **ksi** | MPa | **ksi** | MPa | | | |
| **Example 3 Group 3** | **A** | A1 | 191.5 | 1320.1 | 270.6 | 1865.6 | * | 40.7 | ** |
| | | A2 | 185.1 | 1276.3 | 263.2 | 1814.6 | 11.9 | 43.1 | **21,666** |
| | | **Avg.** | **188.3** | **1298.2** | **266.9** | **1840.1** | **11.9** | **41.9** | **21,666** |
| | | | | | | | | | |
| | **C** | C1 | 167.8 | 1156.9 | 258.7 | 1783.8 | 12.8 | 46.5 | **22,797** |
| | | C2 | 171.4 | 1181.6 | 263.3 | 1815.1 | 11.6 | 17.3 | **21,109** |
| | | **Avg.** | **169.6** | **1169.2** | **261.0** | **1799.4** | **12.2** | **46.9** | **21,953** |
| | | | | | | | | | |
| | **E** | E1 | 171.1 | 1179.7 | 260.7 | 1797.1 | 12.6 | 44.5 | **22,554** |
| | | E2 | 174.7 | 1204.2 | 260.5 | 1796.4 | 13.6 | 46.1 | **24,377** |
| | | **Avg.** | **172.9** | **1191.9** | **260.6** | **1796.8** | **13.1** | **45.3** | **23,465** |

| | | | | | | | | | |
|---|---|---|---|---|---|---|---|---|---|
| * = Invalid measurement - Specimen broke outside gage section ** = No value could be calculated. | | | | | | | | | |

The data presented in Tables 3A-3D, 5, and 6A-6C show that the preferred alloys according to the present invention provide a desirable combination of strength and ductility that makes them uniquely suitable for use in automotive parts made from thin gauge product forms such as strip and sheet. Although one of the specimens was too damaged to be tested and the elongation measurements for some of the specimens were not valid, considered as a whole the data show that the preferred embodiments of the alloy of this invention provide the combination of properties for which the alloy was designed. The unique combination of very high strength and higher than expected ductility, provides a novel solution to the automotive industry for making shaped body and frame parts with reduced weight without sacrificing strength and toughness.

## Claims

1. A steel alloy that provides a unique combination of strength, toughness, and ductility, said alloy consisting essentially of, in weight percent
| | |
|---|---|
| **C** | 0.3-0.45 |
| **Mn** | 3.5-4.5 |
| **Si** | 1.0-2.0 |
| **Cr** | 0.6-2.5 |
| **Ni** | 0.6-5.0 |
| **Mo+½W** | Up to 0.5 |
| **Cu** | 0.3-1.0 |
| **Co** | 0.01 max. |
| **V+5/9Nb** | 0.1-0.5 |
| **Ti** | 0.025 max. |
| **Al** | 0.025 max. |
| **Ca** | 0.005 max. |
| **N** | 0.020 max |
optionally one or both of 0.001-0.025% Y and 0.001-0.01% Mg:
and the balance is iron and the usual impurities, wherein said impurities include not more than about 0.03% phosphorus and not more than about 0.003% sulfur; and wherein the elements Si, Cu, V, and Nb are balanced such that $4.5 \leq \left(%Si+%Cu\right) / \left(%V+\left(5/9\right)\times %Nb\right) \leq 10.$

2. The alloy as claimed in Claim 1 having the following composition ranges, in weight percent, for the respective elements
| | |
|---|---|
| **Si** | 1.3-1.8 |
| **Cr** | 0.75-2.35 |
| **Ni** | 0.7-4.5 |
| **MO+½W** | Up to 0.3 |
| **Cu** | 0.4-0.7 |
| **V+5/9Nb** | 0.2-0.4 |
| **Ti** | 0.020 max. |
| **Al** | 0.020 max. |
| **Ca** | 0.002 max. |

3. The alloy as claimed in Claim 1 having the following composition ranges, in weight percent, for the respective elements
| | |
|---|---|
| **C** | 0.30-0.40 |
| **Si** | 1.3-1.7 |
| **Cr** | 1.6-2.35 |
| **Ni** | 3.7-4.3 |
| **MO+½W** | 0.1 max. |
| **Cu** | 0.4-0.6 |
| **V+5/9Nb** | 0.30-0.40 |
| **Ti** | 0.020 max. |
| **Al** | 0.020 max. |
| **Ca** | 0.002 max. |
and wherein the impurities include not more than about 0.025% phosphorus and not more than about 0.0025% sulfur,
and wherein the elements Mo, Cr, and C are balanced such that $4.25 \leq \left(%Mo+%Cr\right) / \left(%C\right) \leq 7.5 ;$and
the elements Mn and Ni are balanced such that $3.5 \leq % ⁢ Mn + % ⁢ Ni \leq 8.0.$

4. The alloy as claimed in Claim 1 having the following composition ranges, in weight percent, for the respective elements
| | |
|---|---|
| **C** | 0.30-0.36 |
| **Si** | 1.3-1.7 |
| **Cr** | 0.75-1.5 |
| **Ni** | 0.7-2.5 |
| **MO+½W** | 0.15-0.25 |
| **Cu** | 0.4-0.6 |
| **V+5/9Nb** | 0.20-0.30 |
| **Ti** | 0.020 max. |
| **Al** | 0.020 max. |
| **Ca** | 0.002 max. |
and wherein the impurities include not more than about 0.025% phosphorus and not more than about 0.0025% sulfur.

5. The alloy as claimed in any one of the preceding claims wherein (Mo+ ½W) is at least about 0.20%.

6. The alloy as claimed in any of Claims 1, 2, 4, and 5 wherein the elements Mo, Cr, and C are balanced such that 3.5 ≤ (%Mo +% Cr)/(%C) ≤ 7.5.

7. The alloy as claimed in any one of Claims 1, 2, 4, 5, and 6 wherein the elements Mn and Ni are balanced such that 3.5 ≤ %Mn+%Ni ≤ 8.

8. The alloy as claimed in any one of the preceding claims which contains 0.002-0.020% yttrium.

9. The alloy as claimed in any of the preceding claims which contains 0.001-0.006% magnesium.

10. A thin gauge article such as a sheet or a strip, made from the alloy claimed in any of the preceding claims, said thin gauge article having a Strip Index Number of at least 20,000, wherein the Strip Index Number is defined as the product of the ultimate tensile strength in megapascals (MPa) and the percent elongation, and wherein said thin gauge article has a thickness of 0.0229 to less than 6.35 mm.

11. A shaped part made from the thin gauge article claimed in Claim 10.

## Patentansprüche

1. Stahllegierung, die eine einzigartige Kombination aus Festigkeit, Zähigkeit und Duktilität bereitstellt, wobei die Legierung in Gewichtsprozent im Wesentlichen aus Folgendem besteht:
| | |
|---|---|
| **C** | 0,3-0,45 |
| **Mn** | 3,5-4,5 |
| **Si** | 1,0-2,0 |
| **Cr** | 0,6-2,5 |
| **Ni** | 0,6-5,0 |
| **Mo+1/2W** | bis zu 0,5 |
| **Cu** | 0,3-1,0 |
| **Co** | max. 0,01 |
| **V+5/9Nb** | 0,1-0,5 |
| **Ti** | max. 0,025 |
| **Al** | max. 0,025 |
| **Ca** | max. 0,005 |
| **N** | max. 0,020 |
gegebenenfalls eines oder beide von 0,001 bis 0,025 % Y und 0,001-0,01 % Mg;
und der Rest Eisen und die üblichen Verunreinigungen ist, wobei die Verunreinigungen nicht mehr als etwa 0,03 % Phosphor und nicht mehr als etwa 0,003 % Schwefel umfassen; und wobei die Elemente Si, Cu, V und Nb so gewichtet sind, dass $4,5 \leq \left(% Si+% Cu\right) / \left(% V+\left(5/9\right)\times % Nb\right) \leq 10.$

2. Legierung nach Anspruch 1, die die folgenden Zusammensetzungsbereiche in Gewichtsprozent für die entsprechenden Elemente aufweist:
| | |
|---|---|
| **Si** | 1,3-1,8 |
| **Cr** | 0,75-2,35 |
| **Ni** | 0,7-4,5 |
| **Mo+1/2W** | bis zu 0,3 |
| **Cu** | 0,4-0,7 |
| **V+5/9Nb** | 0,2-0,4 |
| **Ti** | max. 0,020 |
| **Al** | max. 0,020 |
| **Ca** | max. 0,002 |

3. Legierung nach Anspruch 1, die die folgenden Zusammensetzungsbereiche in Gewichtsprozent für die entsprechenden Elemente aufweist:
| | |
|---|---|
| **C** | 0,30-0,40 |
| **Si** | 1,3-1,7 |
| **Cr** | 1,6-2,35 |
| **Ni** | 3,7-4,3 |
| **Mo+1/2W** | max. 0,1 |
| **Cu** | 0,4-0,6 |
| **V+5/9Nb** | 0,30-0,40 |
| **Ti** | max. 0,020 |
| **Al** | max. 0,020 |
| **Ca** | max. 0,002 |
wobei die Verunreinigungen nicht mehr als etwa 0,025 % Phosphor und nicht mehr als etwa 0,0025 % Schwefel umfassen
und wobei die Elemente Mo, Cr und C so gewichtet sind, dass $4,25 \leq \left(% Mo+% Cr\right) / \left(% C\right) \leq 7,5 ;$und
die Elemente Mn und Ni so gewichtet sind, dass $3,5 \leq % ⁢ Mn + % Ni \leq 8,0.$

4. Legierung nach Anspruch 1, die die folgenden Zusammensetzungsbereiche in Gewichtsprozent für die entsprechenden Elemente aufweist:
| | |
|---|---|
| **C** | 0,30-0,36 |
| **Si** | 1,3-1,7 |
| **Cr** | 0,75-1,5 |
| **Ni** | 0,7-2,5 |
| **Mo+1/2W** | 0,15-0,25 |
| **Cu** | 0,4-0,6 |
| **V+5/9Nb** | 0,20-0,30 |
| **Ti** | max. 0,020 |
| **Al** | max. 0,020 |
| **Ca** | max. 0,002 |
wobei die Verunreinigungen nicht mehr als etwa 0,025 % Phosphor und nicht mehr als etwa 0,0025 % Schwefel umfassen.

5. Legierung nach einem der vorangegangenen Ansprüche, wobei (Mo+1/2W) zumindest etwa 0,20 % beträgt.

6. Legierung nach einem der Ansprüche 1, 2, 4 und 5, wobei die Elemente Mo, Cr und C so gewichtet sind, dass 3,5 ≤ (% Mo + % Cr) / (% C) ≤ 7,5.

7. Legierung nach einem der Ansprüche 1, 2, 4, 5 und 6, wobei die Elemente Mn und Ni so gewichtet sind, dass 3,5 ≤ % Mn + % Ni ≤ 8.

8. Legierung nach einem der vorangegangenen Ansprüche, die 0,002 bis 0,020 % Yttrium enthält.

9. Legierung nach einem der vorangegangenen Ansprüche, die 0,001 bis 0,006 % Magnesium enthält.

10. Dünner Gauge-Artikel wie z. B. eine Bahn oder ein Streifen, die/der aus einer Legierung nach einem der vorangegangenen Ansprüche hergestellt ist, wobei der dünne Gauge-Artikel eine Strip-Index-Zahl von zumindest 20.000 aufweist, wobei die Strip-Index-Zahl als das Produkt der Grenzzugfestigkeit in Megapascal (MPa) und der prozentuellen Dehnung definiert ist und wobei der dünne Gauge-Artikel eine Dicke von 0,0229 bis weniger als 6,35 mm aufweist.

11. Formteil, das aus dem dünnen Gauge-Artikel nach Anspruch 10 hergestellt ist.

## Revendications

1. Alliage d'acier qui réalise une combinaison unique de résistance, de ténacité et de ductilité, ledit alliage consistant essentiellement, en pourcentages en poids, en :
| | |
|---|---|
| C | 0,3 à 0,45 |
| Mn | 3,5 à 4,5 |
| Si | 1,0 à 2,0 |
| Cr | 0,6 à 2,5 |
| Ni | 0,6 à 5,0 |
| Mo + 1/2W | jusqu'à 0,5 |
| Cu | 0,3 à 1,0 |
| Co | 0,01 au maximum |
| V + 5,9Nb | 0,1 à 0,5 |
| Ti | 0,025 au maximum |
| Al | 0,025 au maximum |
| Ca | 0,005 au maximum |
| N | 0,020 au maximum |
éventuellement l'un ou les deux parmi 0,001 à 0,025 % de Y et 0,001 à 0,01 % de Mg ;
le reste étant du fer et les impuretés habituelles, dans lequel lesdites impuretés ne comprennent pas plus d'environ 0,03 % de phosphore et pas plus d'environ 0,003 % de soufre ; et dans lequel les éléments Si, Cu, V et Nb sont équilibrés de façon que $4,5 \leq \left(%Si+%Cu\right) / \left(%V+\left(5/9\right)\times %Nb\right) \leq 10.$

2. Alliage selon la revendication 1 ayant les plages de composition suivantes, en pourcentages en poids, pour les éléments respectifs :
| | |
|---|---|
| Si | 1,3 à 1,8 |
| Cr | 0,75 à 2,35 |
| Ni | 0,7 à 4,5 |
| Mo + 1/2W | jusqu'à 0,3 |
| Cu | 0,4 à 0,7 |
| V + 5/9Nb | 0,2 à 0,4 |
| Ti | 0,020 au maximum |
| Al | 0,020 au maximum |
| Ca | 0,002 au maximum. |

3. Alliage selon la revendication 1 ayant les plages de composition suivantes, en pourcentages en poids, pour les éléments respectifs :
| | |
|---|---|
| C | 0,30 à 0,40 |
| Si | 1,3 à 1,7 |
| Cr | 1,6 à 2,35 |
| Ni | 3,7 à 4,3 |
| Mo + 1/2W | 0,1 au maximum |
| Cu | 0,4 à 0,6 |
| V + 5/9Nb | 0,30 à 0,40 |
| Ti | 0,020 au maximum |
| Al | 0,020 au maximum |
| Ca | 0,002 au maximum. |
et dans lequel les impuretés ne comprennent pas plus d'environ 0,025 % de phosphore et pas plus d'environ 0,0025 % de soufre ;
et dans lequel les éléments Mo, Cr et C sont équilibrés de façon que $4,25 \leq \left(%Mo+%Cr\right) / \left(%C\right) \leq 7,5 ;$et
les éléments Mn et Ni sont équilibrés de façon que $3,5 \leq % ⁢ Mn + % ⁢ Ni \leq 8,0.$

4. Alliage selon la revendication 1 ayant les plages de composition suivantes, en pourcentages en poids, pour les éléments respectifs :
| | |
|---|---|
| C | 0,30 à 0,36 |
| Si | 1,3 à 1,7 |
| Cr | 0,75 à 1,5 |
| Ni | 0,7 à 2,5 |
| Mo + 1/2W | 0,15 à 0,25 |
| Cu | 0,4 à 0,6 |
| V + 5/9Nb | 0,20 à 0,30 |
| Ti | 0,020 au maximum |
| Al | 0,020 au maximum |
| Ca | 0,002 au maximum. |
et dans lequel les impuretés ne comprennent pas plus d'environ 0,025 % de phosphore et pas plus d'environ 0,0025 % de soufre.

5. Alliage selon l'une quelconque des revendications précédentes, dans lequel (Mo + 1/2W) est d'au moins environ 0,20 %.

6. Alliage selon l'une quelconque des revendications 1, 2, 4 et 5, dans lequel les éléments Mo, Cr et C sont équilibrés de façon que 3,5 ≤ (%Mo + %Cr) / (%C) ≤ 7,5.

7. Alliage selon l'une quelconque des revendications 1, 2, 4, 5 et 6, dans lequel les éléments Mn et Ni sont équilibrés de façon que 3,5 ≤ %Mn + %Ni ≤ 8.

8. Alliage selon l'une quelconque des revendications précédentes, qui contient 0,002 à 0,020 % d'yttrium.

9. Alliage selon l'une quelconque des revendications précédentes, qui contient 0,001 à 0,006 % de magnésium.

10. Article de faible épaisseur tel qu'une feuille ou une bande, fait de l'alliage selon l'une quelconque des revendications précédentes, ledit article de faible épaisseur ayant une valeur d'indice d'enrubannage d'au moins 20 000, laquelle valeur d'indice d'enrubannage est définie par le produit de la résistance à la traction ultime en mégapascals (MPa) et du pourcentage d'allongement, et lequel article de faible épaisseur a une épaisseur de 0,0229 à moins de 6,35 mm.

11. Pièce façonnée faite à partir de l'article de faible épaisseur selon la revendication 10.
